

(No Model.)

E. HERMITE.

BLEACHING OF PAPER PULP OR OTHER FIBROUS OR TEXTILE  
MATERIALS OR FABRICS.

No. 294,619.

Patented Mar. 4, 1884.



WITNESSES:

John D. Parker  
James F. John

INVENTOR:  
Eugene Hermite  
by his Attorneys  
Howson & Sons

# UNITED STATES PATENT OFFICE.

EUGÈNE HERMITE, OF PARIS, FRANCE.

## BLEACHING OF PAPER-PULP OR OTHER FIBROUS OR TEXTILE MATERIALS OR FABRICS.

SPECIFICATION forming part of Letters Patent No. 294,619, dated March 4, 1884.

Application filed December 3, 1883. (No model.) Patented in France October 22, 1883; in Belgium October 29, 1883; in England October 30, 1883; in Austria-Hungary October 30, 1883; in Spain October 30, 1883; in Russia October 31, 1883; in Germany November 3, 1883; in Norway November 3, 1883; in Italy November 8, 1883; in Denmark November 8, 1883; in Sweden November 10, 1883, and in Portugal December 22, 1883.

To all whom it may concern:

Be it known that I, EUGÈNE HERMITE, a citizen of the Republic of France, and residing in Paris, France, have invented certain 5 Improvements in or Connected with the Bleaching of Paper-Pulp or other Fibrous or Textile Materials or Fabrics, of which the following is a specification.

This process may be employed for bleaching 10 textile materials generally, but is more especially applicable to bleaching paper-pulp.

For convenience of description the said process may be considered as divided into two stages.

15 In carrying out the first stage of the improved process, chloride of sodium or of potassium is decomposed by an electric current, and in presence of a metal, preferably lead, in such a manner as to obtain soda and potash 20 and chloride of lead.

The form and arrangement of the apparatus employed may be modified according to circumstances; but good results have been obtained with the apparatus hereinafter described.

25 The view in the accompanying drawing is a sectional view illustrating the apparatus.

In the center of a wooden vessel, A, the bottom of which is provided with a discharge-pipe, a, is placed a porous cylinder, B, on the axis of which is arranged a leaden cylinder, C, forming the negative electrode. A second leaden cylinder, D, surrounding the porous cylinder, acts as the positive electrode. Any 30 convenient number of cells thus constituted are connected in tension.

Underneath the discharge-pipes there is provided a wooden gutter or trough, E, which collects the chloride of lead formed, and conducts it to a tank, F, provided for its reception. A solution of bay salt is prepared in a tank, H, whence it is drawn by a pump, G, and transferred to a store-tank, K, from which it is distributed to the porous vessels and cases. The electric current acts upon the bay salt in the porous vessel, the solution occupying the remaining part of the case, acting more especially as a conducting-liquid. Under the influence of the current chloride of

lead is formed at the positive pole, and caustic 50 soda at the negative pole, (or potash when chloride of potassium is used.) The soda is removed by means of pipes b, extending at one extremity nearly to the bottom of the porous vessels, and connected at the other extremity with a closed chamber, L, from which the liquid is drawn by a pump, M, and delivered into a suitable tank or vessel, N. The soda or potash obtained by this operation is used in the usual manner for bleaching purposes. The chloride of lead serves to produce the chlorine necessary for bleaching the materials prepared by the soda.

55 In carrying out the second stage of the improved process, the chloride of lead obtained by means of the operation hereinbefore described is mixed with water and a small quantity of hydrochloric acid, and subjected to electrolysis in the presence of textile fabrics or materials, or pulp for making paper. When 60 applied to this pulp, the operation is preferably performed in the rag-engine, which is arranged accordingly. The bottom of the trough of the engine is nearly covered by a plate of lead laid in the trough and acting as a 65 negative electrode, upon which the precipitated lead is deposited. Over this is arranged an insulated sheet of wire-gauze. The positive pole, situated above the gauze and insulated therefrom, is constituted by a plate of prepared carbon, platinum, or platinized copper or other conducting material proof against the action of chlorine. At the negative pole any 70 suitable conducting material may be employed in place of the lead. The electric current 75 causes nascent chlorine to be generated at the positive pole, and this chlorine is dissolved in the liquid and bleaches the materials under treatment. At the negative pole is deposited metallic lead, which may be collected for the 80 market, or is preferably employed for decomposing a fresh quantity of alkaline chloride, as hereinbefore described, being thereby reconverted into chloride of lead, and then again treated as hereinbefore described. Caustic 85 soda (or potash) and chloride of lead are thus obtained by means of the improved process. The soda is used to prepare the textile or

fibrous materials in the bleaching process. The gradual and regulated decomposition of the chloride of lead by the electric current in the presence of the fibrous material enables 5 the bleaching to be economically effected without injuring the fibers.

For decomposing the chlorides of potassium or of sodium, zinc, iron, or tin may be employed in place of lead at the positive pole. 10 Caustic soda is thereby obtained, as in the first case, and chlorides of zinc, iron, or tin at the positive pole. The chlorides subjected to electrolysis in presence of the textile or fibrous material yield nascent chlorine, and the metal 15 is deposited as hereinbefore described with reference to lead.

I claim—

1. In bleaching textile or fibrous materials, decomposing chlorides of soda or potash by 20 an electric current under such conditions as to cause the formation of an alkali (soda or potash) and a metallic chloride, preferably

chloride of lead, substantially as hereinbefore described.

2. In bleaching textile or fibrous materials, 25 decomposing the metallic chloride in the presence of the materials that are to be bleached, and recovering the metal in the metallic state for use in subsequent operations, substantially as hereinbefore described.

3. In an apparatus for bleaching fibrous materials, the combination of a rag-engine or equivalent apparatus with the above-described devices for simultaneously effecting the electrolysis of the metallic chloride, bleaching the pulp, and recovering the precipitated metal, substantially as set forth. 30 35

In testimony whereof I have signed my name to this specification in the presence of two subscribing witnesses.

EUGÈNE HERMITE.

Witnesses:

LÉON FRANCKEN,  
ROBT. M. HOOPER.